

June 15, 1937.

C. J. AULBACH ET AL

2,084,070

## METHOD OF COATING CANS

Filed Feb. 13, 1936



Fig. 1.



Fig. 2.



Fig. 3.



Fig. 5.



334  
Charles J. Aulbach,<sup>94</sup>  
Carl A. Herrig,  
Mason & Foster  
Attorneys.

## UNITED STATES PATENT OFFICE

2,084,070

## METHOD OF COATING CANS

Charles J. Aulbach and Earl A. Herrig, Syracuse,  
N. Y., assignors to Continental Can Company,  
Inc., New York, N. Y., a corporation of New  
York

Application February 13, 1936, Serial No. 63,809

1 Claim. (Cl. 91—68)

The invention relates to new and useful improvements in a method of providing a can with a thermoplastic coating such as wax. An efficient way of applying a coating of a thermoplastic material to the interior of a can is to reduce said material to liquid form and flood the interior surface of the can with said material while the can is inverted, and allowing the surplus material to drain from the can. During the draining, the wax adheres to the metal and will flow around on to the under face of the lip of the nozzle, thus producing a relatively thick coating of wax on the outer face of the lip, which is objectionable, for the reason that when the sealing pressure of the gasket is applied thereto, it is likely to craze and cleave from the metal.

An object of the invention is to provide a method whereby the wax accumulating on the outer face of the lip of the can nozzle during draining may be stripped or removed therefrom without, in any way, disturbing the coating covering the edge of the nozzle mouth.

In the drawing—

Figure 1 is a view showing a portion of a can with the wax drained therefrom and also showing the wax collecting on the outer face of the nozzle lip during draining;

Fig. 2 is a view similar to Fig. 1, but showing the wax stripped or removed from the outer face of the nozzle lip;

Fig. 3 is a view showing the nozzle of the can with the wax stripped from the outer face of the lip and the can closed by a crown cap;

Fig. 4 is a view showing more or less diagrammatically and in section a portion of an apparatus which may be used for applying a thermoplastic coating to the interior of the can; and

Fig. 5 is a view showing more or less diagrammatically a portion of an apparatus which may be used for stripping or removing the accumulated wax from the outer face of the nozzle lip.

The improved method has to do with the coating of a can provided with a nozzle which is closed by a cap, and a brief detail description will be given of the can nozzle and the manner of closing the same.

The can which is indicated at 1 is provided with a nozzle 2 having an inturned portion 3 surrounding an opening 4 through which a can may be filled and emptied. The inturned portion 3 at its free edge is turned downwardly and inwardly as indicated at 5. The nozzle is shaped so as to provide a shoulder 6. The can is closed by means of a cap 7 having a sealing gasket 8 disposed within

the same which is adapted to engage the outer face 9 of the nozzle lip. This crown cap is preferably crimped and bent underneath the shoulder 6 as indicated at 10.

The first step in the method consists in the applying of a coating of a thermoplastic material such as wax to the interior of the can. In Fig. 4, there is illustrated one form of apparatus which may be used for accomplishing this result. The can is inverted and is supported during coating by fingers 11 carried by a traveling support 12. A nozzle 13 is raised into the can as it travels for the purpose of supplying the coating material to the interior of the can. The can during travel preferably moves over a coating bath, and means is provided for supplying the nozzle with a coating material in fluid form, under pressure, so that as it flows from the upper end of the nozzle it will flood the entire inner surface of the can and will drain from the nozzle back into the tank. The coating machine which has just been referred to briefly, is shown and described in detail in the application of Alfred L. Kronquest, Serial No. 56,740, filed December 30, 1935. The particular way of coating the can forms no part of the present invention, except for the fact that the can is flooded with the thermoplastic coating material while in liquid form and allowed to drain from the can. As the wax coating drains from the can, it will adhere to the metal and will flow around on to the outer face of the nozzle lip. In Fig. 1 of the drawing, a portion of the nozzle of the can is shown, and the coating is indicated at 14. The portion of the coating adhering to the outer face of the nozzle lip is indicated at 14a.

After the can has been coated and drained sufficiently to leave a proper thickness of coating on the interior of the can, it is then subjected to the next step in the method forming the present invention where this surplus and undesirable coating material 14a on the outer face of the nozzle lip is removed. This is preferably accomplished by placing the can while it is still inverted and the coating material is in flowing form over a pipe 15. The can is so supported on a ledge 16 that the inturned portion of the nozzle 5 forming the nozzle lip is out of contact with the pipe 15. This pipe 15 is mounted on a support 17 and a port 18 formed in the support leads to a vacuum creating means, so that at the proper time, the pipe 15 may be placed under a vacuum pull so that air will be drawn from the can. As the vacuum pull continues, air will flow in between the lip of the nozzle and the outer end of the pipe into the

can and out through the pipe, and this creates a stream of air across the nozzle lip 8.

The stream of air flowing inwardly across the outer face of the nozzle lip will take up the thermoplastic material and carry it along in the air stream. This will gradually thin the coating which accumulated on the outer face of the nozzle lip until it is completely stripped from the outer face, but will leave the coating extending

- 10 from the interior of the nozzle across the edge of the nozzle mouth where it terminates in a very thin edge as indicated at 8a, (Fig. 2). Inasmuch as the nozzle is centered over the pipe and equally spaced therefrom, the stream of air will operate at the same time on all portions of the coating on the nozzle lip, and thus the coating will be quickly stripped from the nozzle. The portion of the apparatus shown in Fig. 5, for removing the coating from the nozzle, is
- 15 shown and described in full in an application of Alfred L. Kronquest and Charles J. Aulbach, Serial No. 57,051, filed December 31, 1935. This apparatus forms no part of the present invention, and is illustrated solely for the purpose of showing one way of carrying out the method.

When the crown cap is applied to the nozzle for closing the can, the sealing gasket 8 contacts with the outer face 9 of the nozzle lip. If the wax was allowed to remain on said outer face, as indicated in Fig. 1, the pressure of the sealing gasket against the wax coating would cause it to crack and when the cap is removed, the wax will cleave off and this, of course, is very objectionable. However, when the wax is stripped

- 20 from the outer face of the nozzle by the method above described, then the sealing gasket contacts directly with the metal at the outer face of the nozzle lip. The gasket will make sufficient contact with the coating at the thinned edge 8a so
- 25 as to prevent the contents of the can reaching the

metal at the outer edge of the lip, and at the same time there will be no destructive pressure of the gasket on the wax coating.

It will be understood, of course, that other means may be provided for applying the coating and the draining thereof from the can, and also for removing or stripping the wax from the outer face of the nozzle lip. The essential features of the invention reside in the method of coating the can with a thermoplastic coating material and allowing the surplus coating material to drain from the can, and then subjecting the outer face of the nozzle lip to an air stream so as to remove or strip all of the wax from said outer face of the nozzle lip. It is essential that the wax shall be in a flowing condition when the air stream is directed across the same, and preferably the operation of removing the wax follows immediately after the coating and draining and before the wax takes on a set condition.

Having thus described the invention, what we claim as new and desire to secure by Letters Patent, is—

The method of coating cans, having a nozzle provided with a lip, with a thermoplastic material consisting in flowing the coating material while in liquid form over the inner surface of the can, draining the surplus material therefrom, placing said can while the coating is in flowing form over a pipe in alignment with the center of the nozzle and with the nozzle lip spaced a short distance from the end of the pipe and connecting said pipe to a vacuum creating means for drawing air through the pipe and across the face of the lip of the nozzle for removing the coating collecting thereon during draining.

CHARLES J. AULBACH.  
EARL A. HERRIG.